# EUROPEAN PATENT SPECIFICATION

(11) **EP 0 006 957 B1**
(45) Date of publication and mention of the grant of the patent: **03.10.1984**
(21) Application number: 78900302.7
(22) Date of filing: 14.11.1978
(51) Int. Cl.: B21D 51/26, B65D 25/14, C10M 3/20

(54) **METHOD OF MAKING METAL CONTAINERS**
VERFAHREN ZUR HERSTELLUNG VON METALLBEHÄLTERN
METHODE DE FORMATION DE BOITES SANS COUTURE

(30) Priority: 16.11.1977 US 851856; 16.11.1977 US 851859
(43) Date of publication of application: 23.01.1980
(73) Proprietor: AMERICAN NATIONAL CAN COMPANY, Chicago Illinois 60631 (US)
(72) Inventor: MISRA, Surya, K., Naperville, IL 60540 (US); OPENCHOWSKI, Richard, A., Woodridge, IL 60515 (US); ZENGER, Richard, D., Downers Grove, IL 60515 (US); HESSEL, William, Darien, IL 60559 (US)
(74) Representative: Bowtell, Peter Lloyd
(86) International application number: US7800146
(87) International publication number: WO7900297

## Description

### Background of the Invention

The present invention relates generally to containers and more particularly to an improved stock material for making containers and a method for forming seamless drawn and ironed containers from the improved stock material.

The use of a two-piece container for packaging beer and/or carbonated beverages has become very popular in recent years. The two-piece container consists of a container sidewall or body that has a unitary end wall at one end thereof. The second piece for the containercon- sists of an end which is seamed to the open end of the container.

In the formation of drawn and ironed containers, a finished container is produced by initially cutting a disc from a sheet or coil of stock material and substantially simultaneously transforming the disc into a shallow cup in a conventional cupping machine that forms part of a can manufacturing line. The shallow cup is then converted into a drawn and ironed container in a body maker wherein the shallow cup is reformed into a cup of different dimensions and then passed through a plurality of ironing rings that cooperate with a punch to decrease the wall thickness of the reformed cup and produce a seamless container. Alternatively, the cup may initially have a diameter substantially equal to the final diameter so that the reforming or redrawing in the body maker is not necessary.

In most commercial machinery utilized for forming the cups and then converting the cups to drawn and ironed containers, a lubricant-coolant is utilized in the cupper for providing the necessary lubricity between the surface of the stock material and the tooling. The body making machinery also incorporates mechanism for flowing a lubricant-coolant to the surface of the container and to the ironing dies utilized in cooperation with the punch. Conventionally, the lubricant-coolant consists of a mixture of water and an emulsified oil or emulsified synthetic lubricant, such as a commercially available Texaco 591 product. One of the difficulties with utilizing the water soluble emulsified oils in the cupping as well as the drawing and ironing tooling is subsequent cleaning of the finished containers to remove the emulsified oils from the surfaces thereof. In order to produce an acceptable surface that can subsequently be coated and/or decorated, it is necessary to utilize harsh chemicals and washing temperatures as high as 72°C to remove the undesired emulsified oils. Furthermore, it has been determined that some emulsified oils may become toxic which presents a potential health hazard.

Presently, most drawn and ironed containers are formed from aluminum because of the relative ease in fabricability of the container. Because of the cost of aluminum, manufacturers are constantly striving to find an acceptable substitute for aluminum which can be manufactured at a competitive cost.

One acceptable alternative for the drawn and ironed aluminum container is commonly referred to as tinplate. This material includes a base plate of low carbon steel, such as black plate which has both surfaces covered with a thin layer of tin. The tin coating acts as low friction, ductile material during the ironing process and also resists corrosion. While tinplate has been found to be an acceptable alternative for aluminum, the availability of this material is limited and the cost is high.

Bethlehem Steel Corporation also has continued its development efforts for producing a beer and carbonated beverages container from black plate using conventional machinery by applying organic coating to the black plate which can then be drawn and ironed at a price which is competitive to the present day tinplate or aluminium container. To this end, a proposed process is disclosed in United States Patent No. 4,032,678.

This process contemplates the formation of polymeric thermosetting coating systems that enable container manufacturers to produce drawn and ironed beer and soft-drink cans from black plate. The foregoing patent describes two coating concepts that have been developed for black plate, one of which consists of admixing a thermosetting coating and a lubricant and applying this mixture to both sides of the black plate blank and partially curing the mixture before the blank is converted into a finished container. The other concept contemplates supplying the coating-lubricant mixture to only the one side of the blank (the side forming the outside of the can), and applying a coating lubricant alone to the other side of the blank (the side that forms the inside of the can). Actual tests carried out using such polymeric thermosetting coatings show that containers formed from such coated black plate, but without having an internal lubricant mixed with the coating, retained substantially more coating on the finished container than when the internal lubricant was present in the coating.

Also, while such process as described in U.S. Patent No. 4032678 is acceptable in laboratory trials at slow speeds, actual tests have shown that the partially-cured coating having the lubricant mixed therein, while allowing drawing and ironing of the container, is not acceptable for making cans at commercial production rates and most of the coating is removed during the ironing process when containers are manufactured at rates of more than 150 containers per minute.

It was also determined that the coating was removed in the form of large flakes or long narrow strips which would be introduced into the coolant and would rapidly clog up the filtering system for the coolant. These flakes or strips would also be carried by the container to downstream areas of the container processing line which disrupted the proper processing of the containers.

Accordingly the present invention provides a method of forming a seamless container having a bottom wall and an integral sidewall from metal stock material by cutting a disc from said stock material, drawing said disc into a cup and substantially reducing said sidewall of said cup in a multi-stage ironing process to produce a drawn and ironed container, characterised by applying a thin layer of a lubricant only of between 0.2 mg/cm² and 0.5 mg/cm² to at least one surface of said stock material before said disc is cut out from said stock material, said lubricant consisting of only an ester of a monomeric polyhydric alcohol having 3 to 6 hydroxyls and a 14 to 20 carbon fatty acid, and forming said seamless drawn and ironed container with at least some of said lubricant remaining on said surface throughout said multi-stage ironing process.

Thus in the method of the present invention, a metal base of stock material that is to be used for forming a drawn and iron seamless container first has a thin layer of lubricant applied to at least one surface of the metal stock or blank and a disc is cut from the metal blank and formed into a shallow cup without the use of any additional lubricant or coolant. The shallow cup is then further drawn and ironed to produce a seamless container which again is done without the use of any additional lubricant in the liquid coolant, such as water, in the drawing and ironing machine.

It has been determined that all lubricants in the cooling fluid can be eliminated by applying a thin layer of an organic ester to the stock material before the cupping operation is initiated and that applying a single layer of lubricant consisting of only a fatty acid ester as defined above of less than 0.5 mg/cm² even to one surface only of black plate, tinplate or aluminium by a commercial lubricator eliminates the need for any subsequent lubrication in the cupping machine as well as the body maker.

### Description of the Invention

In its broadest aspect, the present invention contemplates precoating a metal sheet or coil with a thin layer of lubricant to the metal sheet or coil, cutting a disc from the metal sheet or coil with the lubricant applied to it, forming a shallow cup from the disc, subsequently redrawing and ironing the shallow cup into a full sized container.

Stated another way, a stock material, such as an aluminium, black plate or tinplate metal sheet or coil, has a layer of lubricant consisting only of a fatty acid ester as defined above, applied to a surface of the stock material to a thickness of between 0.2 mg/cm² (1 mg/in²) and 0.5 mg/cm² (3 mg/in²) and preferably about 0.2 mg/cm² (1 mg/in2) and the pretreated stock material is then utilised in forming a seamless drawn and ironed container that has a bottom wall and an integral sidewall in conventional cupping and body making machinery that is presently utilized for making such containers. By applying the lubricant to the stock material before a disc is cut therefrom, all additional lubricants in the drawing and ironing process may be eliminated in the preferred embodiment making subsequent operations such as cleaning easier. The body maker may be provided with a water coolant that has a small amount of rust inhibitor therein to maintain the tooling below a predetermined temperature.

A commercially available ester lubricant made from a monomeric polyhydric alcohol having three to six hydroxyls and a 14 to 20 carbon fatty acid suitable for use in the present invention is produced by Mobil Chemical Company under the designation S-6661-003.

The Mobil lubricant was successfully applied to one surface of black plate, tinplate and aluminium plate by a lubricator to produce a thin layer of lubricant having a thickness or distribution of less than 0.5 mg/cm² (3 mg/in²) on the surface of the stock material that ultimately becomes the inside of the container. If necessary, to produce the desired thickness of the layer, it may be necessary to either thin the fatty acid ester with a solvent before it is applied to the surface of the stock material, or simply by heating the material before it is applied by the lubricator. A further alternative form of heating would be to heat the rollers that form part of the lubricator.

The invention may be carried into practice in various ways and a number of Examples will now be described by way of example.

### Example I

Laboratory tests were conducted by applying a layer of approximately 0.2 mg/cm² (1.25 mg/in²) of the above Mobil lubricant on one surface of a sheet of tinplate stock material. The sheet of stock material was then cut and formed into shallow cups in a conventional manner without the addition of any further lubricant or without any water. The cups with the layer of lubricant on the inner surface, were then reformed into finished containers in a conventional body maker where only water alone or water with 0.05% rust inhibitor was circulated through the tooling used in producing the finished container. Some containers were made using a water-emulsion oil mixture for the coolant.

Containers made using a lubricant consisting of only a fatty acid ester as defined above pre- applied to sheets or coils consistently showed better cleanability when water alone was used as the coolant. In all instances the containers made without the emulsion oil lubricant had a smooth and uniform surface appearance.

### Example II

Aluminium stock material in the form of plates was coated on one side with a lubricant consisting of only a fatty acid ester, such as the Mobil lubricant, to produce a layer on one surface having a distribution of approximately 0.2 mg/cm² (1.25 mg/in²). These plates were then converted into cups and subsequently cans utilizing a commercially available cupper and body maker. In converting the plates into cups, the plates were positioned so that the lubricated surface became the internal surface of the cup and no additional lubricant or water was needed to produce satisfactory cups from the plates. The cups were then converted to finished containers in the body maker utilizing only tap water. Several thousand of such cups and containers were produced and inspection of the finished containers showed that the containers had a shiny outside surface and a scratch-free inside surface. The containers were then cleaned using several standard cleaners with less than the present standard recommended concentration to remove all of the lubricants from the container surfaces.

The above tests establish that drawn and ironed containers can be formed from coated black plate, aluminium or tinplate by precoating the stock material with a thin layer of a lubricant consisting of only a fatty acid ester as defined above and the drawn and ironed containers can be formed without the use of water or emulsifiable oils in the cupper and using only water as a coolant in the body maker or drawing and ironing machine.

It is believed that elimination of the water emulsion oils from the process and substitution of a lubricant consisting of only a fatty acid ester as defined above results in a cost saving of approximately 50% in the lubricant alone and also provides additional savings in the use of milder cleaners and lower cleaning temperatures.

It has also been established that the lubricant consisting of only a fatty acid ester as defined above provides better lubrication for the tooling than the water-lubricant mixture. This is believed to result from the fact that the lubricant is initially located directly between the tooling and the container surface interface and also from the fact that the lubricant consisting of only a fatty acid ester as defined above withstands the high temperature encountered during ironing of the metal body without deterioration. Also, applying the layer of lubricant to the surface which becomes the inner surface of the container is believed to aid in stripping the ironed container from the punch.

Of course, if desired, both surfaces of the stock material could be coated with a lubricant and/or the distribution or thickness of the layer or layers could be increased. However, tests have shown that increasing the thickness of the coating on one surface only will not increase the efficiency of the operation but will increase the cost without any additional benefits. Respecting the two-sided coating with lubricant, it was determined that the additional coating on the second side increased the costs without deriving any benefits from the increased cost. In other words, tests showed that one side coated material would have enough lubricant transferred to the other side during the processing of the stock material and in the cupper and body maker to eliminate the need for applying lubricant to the second side.

While the manner of applying the lubricant to the stock material is not critical in carrying out the present invention, the lubricant is preferably applied as the stock material is fed to the cupping machine. Of course, the lubricant could also be applied in other ways.

## Claims

1. A method of forming a seamless container having a bottom wall and an integral sidewall from metal stock material by cutting a disc from said stock material, drawing said disc into a cup and substantially reducing said sidewall of said cup in a mult-stage ironing process to produce a drawn and ironed container, characterised by applying a thin layer of a lubricant only of between 0.2 mg/cm² and 0.5 mg/cm² to at least one surface of said stock material before said disc is cut out from said stock material, said lubricant consisting of only an ester of a monomeric polyhydric alcohol having 3 to 6 hydroxyls and a 14 to 20 carbon fatty acid, and forming said seamless drawn and ironed container with at least some of said lubricant remaining on said surface throughout said multi-stage ironing process.

2. A method as defined in Claim 1, characterised by said layer of lubricant having a thickness of approximately 0.2 mg/cm².

3. A method as defined in any one of Claims 1 to 2, characterised in that said metal is aluminium.

4. A method as defined in any one of Claims 1 to 2, characterised in that said metal stock material is tinplate.

5. A method as defined in any one of Claims 1 to 4, in which said metal stock material is a coil of stock material and the layer of lubricant is applied to one surface only of said stock material.

6. A method as claimed in any of the preceding claims in which the layer of lubricant is applied to one surface only of the stock material and is transferred to the other surface during processing of the stock material.

7. A method as defined in any one of Claims 1 to 6 in which said disc is drawn into a cup without any liquid coolant being supplied to said disc.

8. A method as defined in any one of Claims 1 to 6, further including use of a liquid coolant while a drawn and ironed container is being formed.

9. A method as defined in Claim 8 in which the drawing and ironing is done without the use of any additional lubricant in the liquid coolant.

10. A method as defined in any one of Claims 1 to 9 in which said one surface with said lubricant is the inside of said cup.

## Patentansprüche

1. Verfahren zum Bilden eines nahtlosen Behälters mit einer Bodenwand und einer integralen Seitenwand aus Metall-Vorratsmaterial durch Ausschneiden einer Scheibe aus dem Vorratsmaterial, Ziehen der Scheibe zu einem Becher und erhebliches Reduzieren der Seitenwand des Bechers in einem mehrstufigen Weiterschlagprozeß zum Erzeugen eines im Anschlag und Weiterschlag gezogenen Behälters, dadurch gekennzeichnet, daß auf mindestens eine Oberfläche des Vorratsmaterials vor dem Ausschneiden der Scheibe eine dünne Schicht eines Schmiermittels von nur zwischen 0,2 mg/cin² und 0,5 mg/cm² aufgebracht wird, wobei das Schmiermittel nur aus einem Ester eines monomeren mehrwertigen Alkohols mit 3 bis 6 Hydroxylgruppen und einer Fettsäure mit 14 bis 20 Kohlenstoffatomen besteht, und daß beim Bilden des nahtlosen, im Anschlag und Weiterschlag tiefgezogenen Behälters mindestens etwas von dem genannten Schmiermittel während des ganzen mehrstufigen Weiterschlagprozesses auf der genannten Oberfläche verbleibt.

2. Verfahren nach Anspruch 1, dadurch gekennzeichnet, daß die Schmiermittelschicht eine Dicke von etwa 0,3 mg/cm² hat.

3. Verfahren nach Anspruch 1 oder 2, dadurch gekennzeichnet, daß das Metall Aluminium ist.

4. Verfahren nach Anspruch 1 oder 2, dadurch gekennzeichnet, daß das Metall-Vorratsmaterial Zinnblech ist.

5. Verfahren nach einem der Ansprüche 1 bis 4, dadurch gekennzeichnet, daß das Metall-Vorratsmaterial ein Wickel aus Vorratsmaterial ist und daß die Schmiermittelschicht nur auf eine Seite des Vorratsmaterials aufgebracht wird.

6. Verfahren nach einem der vorhergehenden Ansprüche, dadurch gekennzeichnet, daß die Schmiermittelschicht nur auf eine Seite des Vorratsmaterials aufgebracht und während der Verarbeitung des Vorratsmaterials auf die andere Seite übertragen wird.

7. Verfahren nach einem der Ansprüche 1 bis 6, dadurch gekennzeichnet, daß die Scheibe ohne ihr irgendein flüssiges Kühlmittel zuzuführen zu einem Becher tiefgezogen wird.

8. Verfahren nach einem der Ansprüche 1 bis 6, dadurch gekennzeichnet, daß während der Bildung des im Anschlag und im Weiterschlag tiefgezogenen Behälters ein flüssiges Kühlmittel verwendet wird.

9. Verfahren nach Anspruch 8, dadurch gekennzeichnet, daß das Tiefziehen im Anschlag und Weiterschlag ohne Verwendung irgendeines zusätzlichen Schmiermittels im flüssigen Kühlmittel durchgeführt wird.

10. Verfahren nach einem der Ansprüche 1 bis 9, dadurch gekennzeichnet, daß die eine Seite mit dem Schmiermittel die Innenseite des Bechers ist.

## Revendications

1. Procédé de formage de containeur sans soudure présentant une paroi de fond et une paroi latérale qui en fait partie intégrante, fait de métal comme matière première, en découpant un disque dans ladite matière première, puis en étirant ledit disque pour en faire une coupe et en réduisant essentiellement ladite paroi latérale de ladite coupe au cours d'une opération fractionnée d'estampage pour produire un conteneur embouti et estampé, caractérisé par l'application d'une mince couche de lubrifiant uniquement entre 0,2 mg/cm² et 0,5 mg/cm², sur une surface au moins de ladite matière première avant le découpage dudit disque dans ladite matière première, ledit lubrifiant consistant seulement en un ester d'un alcool poly- hydrique monomère ayant 3 à 6 hydroxyles et un acide gras de 14 à 20 atmoes de carbone, et par formage dudit conteneur sans soudure étiré et estampé avec un peu au moins dudit lubrifiant restant sur ladite surface au cours du processus d'estampage en plusieurs étapes.

2. Procédé selon la revendication 1, caractérisé en ce que ladite couche de lubrifiant présente une épaisseur approximative de 0,2 mg/cm².

3. Procédé selon l'une des revendications 1 ou 2, caractérisé en ce que ledit métal est de l'aluminium.

4. Procédé selon l'une des revendications 1 et 2, caractérisé en ce que ledit métal utilisé comme matière première est du fer-blanc.

5. Procédé selon l'une des revendications 1 à 4 dans laquelle ledit métal utilisé comme matère première est un rouleau de métal et où la couche de lubrifiant n'est appliquée qu'à une seule surface de ladite matière première.

6. Procédé selon l'une des revendications précédentes, dans lequel la couche de lubrifiant est appliquée à une seule surface de la matière première et est transférée à l'autre surface pendant le traitement de la matière première.

7. Procédé selon l'une des revendications 1 à 6 dans lequel ledit disque est embouti sous forme de coupe sans qu'aucun liquide de refroidissement ne soit fourni audit disque.

8. Procédé selon l'une des revendications 1 à 6, qui comporte en outre l'utilisation d'un liquide de refroidissement pendant la formation d'un conteneur embouti estampé.

9. Procédé selon la revendication 8, dans lequel l'emboutissage et l'estampage s'effectuent sans utiliser aucun lubrifiant supplémentaire dans le liquide de refroidissement.

10. Procédé selon l'une des revendications 1 à 9, dans lequel ladite première surface pourvue dudit lubrifiant se trouve à l'intérieur de ladite coupe.
